# EUROPEAN PATENT SPECIFICATION

(11) **EP 0 766 131 B1**
(45) Date of publication and mention of the grant of the patent: **08.12.1999**
(21) Application number: 96202665.4
(22) Date of filing: 24.09.1996
(51) Int. Cl.: G03C 1/26, G03C 1/28, G03C 1/29, G03C 1/34, G03C 1/08, G03C 1/09, G03C 7/30

(54) **Photographic material having a red sensitized silver halide emulsion layer with improved heat sensitivity**
Photographisches Material mit einer rot sensibilisierten Silberhalogenidemulsionschicht verbesserter Wärmeempfindlichkeit
Matériau photographique à couche d'émulsion à l'halogénure d'argent sensibilisée à la lumière rouge ayant une sensibilité à la chaleur améliorée

(30) Priority: 29.09.1995 US 4514; 08.04.1996 US 629419
(43) Date of publication of application: 02.04.1997
(73) Proprietor: EASTMAN KODAK COMPANY, Rochester, New York 14650-2201 (US)
(72) Inventor: Garnsey, Richard Paul, Rochester, New York 14650-2201 (US); Ferguson, Pamela McCue, Rochester, New York 14650-2201 (US); Parton, Richard Lee, Rochester, New York 14650-2201 (US); Hahm, Paul Timothy, Rochester, New York 14650-2201 (US)
(74) Representative: Haile, Helen Cynthia

(56) References cited:
- EP-A- 0 336 426
- EP-A- 0 367 227
- EP-A- 0 476 604
- EP-A- 0 605 917
- WO-A-92/12462

## Description

### Field of the Invention

This invention relates to a photographic material having a red sensitized silver halide emulsion layer with improved heat sensitivity.

### Background of the Invention

There is a great emphasis on high productivity in the photosensitive materials market. Photofinishers that use photosensitive paper to produce color prints desire short processing times in order to increase output. One way to obtain rapid processing is to accelerate the development time by increasing the chloride content of the emulsions; the higher the chloride content the higher the development rate. However, it is also known that the higher the chloride content is, the harder it is to obtain high, invariant photosensitivity. Emulsions that are primarily silver chloride are more difficult to spectrally sensitize than emulsions used previously such as silver bromide or chlorobromide emulsions because the conduction band of silver chloride is higher than that of silver bromide (C. R. Berry, Photo. Sci. & Eng. 19, 93, (1975)).

The problem with sensitizing efficiency is especially true in the red-sensitive layer of many color print photosensitive materials and is related to the red sensitizers reduction potential. Correlations between dye reduction potentials and sensitizing efficiency on high silver chloride emulsions are discussed by W. Vanassche, J. Photo. Sci., 21, 180 (1973) and P. B. Gilman, Jr., Photo. Sci. & Eng. 18, 475 (1974). Another common problem with the red sensitive layer of color print paper which contains an emulsion that is primarily silver chloride, is an undesirable sensitivity to temperature. An increase in temperature of the paper during exposure results in an increase in red speed of the red sensitive layer making it difficult for the photofinisher to adjust his printing conditions. This results in a loss in operating efficiency.

An example of heat sensitivity is illustrated below. Material C has no propensity for heat sensitivity while Material A and B have equal propensity but in opposite directions. Color photographic materials typically respond to three regions of the spectrum, red, green and blue with different emulsions and, as an example for color positive paper such as EKTACOLOR Paper, will produce cyan, magenta and yellow dye images when processed in Process RA-4. If the paper temperature changes during the day as it is printed such as due to changing ambient conditions or warming up in the printing environment, the prints can change in density causing a variability in the image produced. With color products a mis-match in the heat sensitivity response of the three layers results in a color shift in the prints. So, while it would be useful to have low heat sensitivity to preserve color consistency in printing, it is more important with color products to have a consistent heat sensitivity shift in all three layers to avoid a shift in the more critical area of color balance. Almost all of the materials used to prepare silver halide emulsions can under some conditions affect the heat sensitivity of the resulting photographic materials. It is therefore desirable to have the ability to adjust the heat sensitivity of a particular emulsion to the appropriate level to match the other two layers.

| | Speed (Log E) of Materials at 22^{o}C | Speed (Log E) of Materials at 40^{o}C | Heat Sensitivity (Delta Log E) |
|---|---|---|---|
| Material A | 1.90 | 2.00 | +.10 |
| Material B | 2.00 | 1.90 | -.10 |
| Material C | 1.90 | 1.90 | 0.00 |

European published patent application EP-A-O 605,917 A2 describes red dyes that give high speed and reduced heat sensitivity when used on high chloride emulsions. However, by the use of these red sensitizers, the heat sensitivity of the cyan layer is so low that it no longer matches that of the magenta and yellow records. This causes an undesirable color balance shift during thermal changes. It is therefore desirable to provide a means of adjusting the heat sensitivity in the cyan layer so as to match that of the magenta and yellow layers. It is toward this end that this invention is directed.

### Problem to be Solved by the Invention

The prior art teaches the use of red dyes that give reduced heat sensitivity. But there is no teaching on how to use these dyes so that the heat sensitivity of the red layer matches that of the magenta and yellow records and thus to avoid heat induced changes in color balance.

### Summary of the Invention

This invention relates to a silver halide photographic material comprising a red sensitive silver halide emulsion layer, the silver halide of which comprises silver halide grains prepared in the presence of a hexacoordination complex of rhenium, ruthenium or osmium with at least four cyanide ligands and comprising at least 90 mole percent silver chloride, wherein the emulsion contains a thiosulfonate compound and a sulfinate or seleninate compound and a dye of Class A and/or Class B:
where,
Class A dyes have structure I and substituents W₁-W₈, are chosen such that J is ≥ 0.0, where J is defined as the sum of the Hammett σₚ values of W₁-W₈, or, alternatively, Class A dyes can also have the structure II provided substituents W₁-W₈ are chosen such that J is ≥ 0.24;
Class B dyes have structure II and substituents W₁-W₈ are chosen independently such that J is ≤ 0.10, or, alternatively, Class B dyes can also have structure I provided substituents W₁-W₈ are chosen such that J is ≤ -0.14 where,
   R₁ and R₂ each independently represent an alkyl group or a substituted alkyl group;
   X is a counterion, if needed, to balance the charge of the dye;
   Z is a hydrogen or halogen atom or an alkyl group or a substituted alkyl group;
   Z₁ and Z₂ are each independently a 1-8 carbon alkyl group;

### Advantageous Effect of the Invention

The present invention provides photographic materials with a high silver chloride layer having high red sensitivity while at the same time having relatively low thermal sensitivity. A method is described to adjust the heat sensitivity of the cyan layer so as to match that of the magenta and yellow layers to maintain color balance despite thermal fluctuations.

### Detailed Description of Embodiments of the Invention

In the present application, by reference to "under", "above", "below", "upper" or "lower" terms in relation to layer structure of a photographic element, is meant in this application, the relative position in relation to light to when the element is exposed in a normal manner. "Above" or "upper" would mean closer to the light source when the element is exposed normally, while "below" or "lower" would mean further from the light source. Since a typical photographic element has the various layers coated on a support, "above" or "upper" would mean further from the support, while "below" or "under" would mean closer to the support.

When reference in this application is made to a substituent "group", this means that the substituent may itself be substituted or unsubstituted (for example "alkyl group" refers to a substituted or unsubstituted alkyl). Generally, unless otherwise specifically stated, substituents on any "groups" referenced herein or where something is stated to be possibly substituted, include the possibility of any groups, whether substituted or unsubstituted, which do not destroy properties necessary for the photographic utility. It will also be understood throughout this application that reference to a compound of a particular general formula includes those compounds of other more specific formula which specific formula falls within the general formula definition. Examples of substituents on any of the mentioned groups can include known substituents, such as: halogen, for example, chloro, fluoro, bromo, iodo; alkoxy, particularly those with 1 to 6 carbon atoms (for example, methoxy, ethoxy); substituted or unsubstituted alkyl, particularly lower alkyl (for example, methyl, trifluoromethyl); alkenyl or thioalkyl (for example, methylthio or ethylthio), particularly either of those with 1 to 6 carbon atoms; substituted and unsubstituted aryl, particularly those having from 6 to 20 carbon atoms (for example, phenyl); and substituted or unsubstituted heteroaryl, particularly those having a 5 or 6-membered ring containing 1 to 3 heteroatoms selected from N, O, or S (for example, pyridyl, thienyl, furyl, pyrrolyl); and others known in the art. Alkyl substituents may specifically include "lower alkyl", that is having from 1 to 6 carbon atoms, for example, methyl or ethyl. Further, with regard to any alkyl group, alkylene group or alkenyl group, it will be understood that these can be branched or unbranched and include ring structures.

The silver halide emulsion can be prepared as described in U.S. Patent No. 4,945,035 of Keevert et al. The silver halide emulsion is a "high chloride" emulsion containing at least 90 mole percent chloride, preferably at least 95 mole percent chloride and optimally at least 98 mole percent chloride. Some silver bromide may be present; in particular, the possibility is also contemplated that the silver chloride could be treated with a bromide source to increase its sensitivity, although the bulk concentration of bromide in the resulting emulsion will typically be no more than 2 to 2.5 mole percent and preferably between 0.6 to 1.2 mole percent (the remainder being silver chloride). The emulsion should contain less than 5 mole percent iodide, preferably less than 2 mole percent iodide.

The preferred hexacoordinated rhenium, ruthenium, and osmium cyanide complexes can be represented by the following formula:

[Q(CN)_{6-y}L_{y}]⁻ⁿ

where:
Q is rhenium, ruthenium, or osmium,
L is a bridging ligand,
y is 0, 1, or 2,
   and
-n is -2, -3, or -4.

The bridging ligand is preferably a monoatomic monodentate ligand, such as a halide, for example, fluoride, chloride , bromide or iodide ligands, or a multielement ligand, for example, azide or thiocyanate ligands. In a particularly preferred embodiment, Q is ruthenium and y is 0.

The hexacoordinated complexes in most instances exhibit a net ionic charge. One or more counter ions are therefore usually associated with the complex to form a charge neutral compound. The counter ion is of little importance, since the complex and its counter ion or ions dissociate upon introduction into an aqueous medium, such as that employed for silver halide grain formation. Ammonium and alkali metal counter ions are particularly suitable for anionic hexacoordinated complexes, since theses cations are known to be fully compatible with silver halide precipitation procedures.

Table I provides a listing of illustrative rhenium, ruthenium, and osmium cyanide coordination complexes.

**TABLE I**

| | |
|---|---|
| [Re(CN)₆]⁻⁴ | [OsF₂(CN)₄]⁻⁴ |
| [Ru(CN)₆]⁻⁴ | [ReCl₂(CN)₄]⁻⁴ |
| [Os(CN)₆]⁻⁴ | [RuCl₂(CN)₄]⁻⁴ |
| [ReF(CN)₅]⁻⁴ | [OsCl₂(CN)₄]⁻⁴ |
| [RuF(CN)₅]⁻⁴ | [ReBr₂(CN)₄]⁻⁴ |
| [OsF(CN)₅]⁻⁴ | [RuBr₂(CN)₄]⁻⁴ |
| [ReCl(CN)₅]⁻⁴ | [OsBr₂(CN)₄]⁻⁴ |
| [RuCl(CN)₅]⁻⁴ | [RuI₂(CN)₄]⁻⁴ |
| [OsCl(CN)₅]⁻⁴ | [OsI₂(CN)₄]⁻⁴ |
| [ReBr(CN)₅]⁻⁴ | [Ru(CN)₅(OCN)]⁻⁴ |
| [RuBr(CN)₅]⁻⁴ | [Os(CN)₅(OCN)]⁻⁴ |
| [OsBr(CN)₅]⁻⁴ | [Ru(CN)₅(SCN)]⁻⁴ |
| [ReI(CN)₅]⁻⁴ | [Os(CN)₅(SCN)]⁻⁴ |
| [RuI(CN)₅]⁻⁴ | [Ru(CN)₅(N₃)]⁻⁴ |
| [OsI(CN)₅]⁻⁴ | [Os(CN)₅(N₃)]⁻⁴ |
| [ReF₂(CN)₄]⁻⁴ | [Ru(CN)₅(H₂O)]⁻³ |
| [RuF₂(CN)₄]⁻⁴ | [Os(CN)₅(H₂O)]⁻³ |

The hexacoordination complex is preferably utilized in an amount of 1 X 10⁻⁶ mole of complex per mole of silver in the emulsion. The complex can be incorporated into the grains up to its solubility limit, typically 5 X 10⁻⁴ mole per silver mole. An excess of the complex over its solubility limit in the grain can be tolerated, but normally any such excess is removed from the emulsion during washing. Preferred concentrations of the complex are from 10⁻⁵ to 10⁻⁴ mole per silver mole.

The emulsion also contains a thiosulfonate compound and a sulfinate or seleninate compound. The thiosulfonate compound is preferably a compound of formula (IV):

T¹―SO₂S―Y¹ (IV)

and the sulfinate compound is preferably a compound of formula (Va):

T²―SO₂―Y² (Va)

and the seleninate compound is preferably a compound of formula (Vb)

T²―SeO₂―Y² (Vb)

wherein:
Y¹ and Y² are independently selected from the group consisting of a metal ion and wherein D₁, D₂, D₃, and D₄ are independently selected from the group consisting of hydrogen and an alkyl of 1-3 carbon atoms, and T¹ and T² are independently selected from the group consisting of an unsubstituted or substituted alkyl of 1 to 22 carbon atoms, an alkenyl of 2 to 22 carbon atoms, an alkynyl of 2 to 22 carbon atoms, an unsubstituted or substituted aryl group having 6 to 20 carbon atoms, an unsubstituted or substituted 5 to 15-membered heterocyclic group having one or two heteroatoms and a divalent linking group. Examples of suitable aryl groups are phenyl, tolyl, naphthyl, and of suitable alkenyl groups are cycloheptatrienyl, cyclooctatrienyl, and cyclononatrienyl. Examples of suitable heterocyclic groups are pyrrolyl, furanyl, tetrahydrofuranyl, thiofuranyl, pyridino, picolino, piperidino, morpholino, pyrrolidino, thiophene, oxazole, thiazole, imidazole, selenazole, tellurazole, triazole, tetrazole and oxadiazole. Examples of suitable divalent linking groups are -(CH(CH₂)ₘ- where m is 1 to 11, -(CH-CH=CH-CH₂)- and -(C(CH₃)CH₂)-. When T¹ or T² is a divalent linking group, the compound of formula (IV), (Va) or (Vb), respectively, is polymeric, with the repeating unit being of formula (IV), (Va), or (Vb), respectively.

In a preferred embodiment Y¹ and Y² are independently selected from Na⁺, K⁺ and and T¹ and T² are independently selected from an unsubstituted phenyl group or a phenyl group substituted in one or two positions independently selected from the group consisting of an alkyl having 1 to 10 carbon atoms, an alkoxy having 1 to 10 carbon atoms, an acyl having 1 to 10 carbon atoms, an hydroxyl, a phenyl, a tolyl, a naphthyl, a carboxy, a chloro, a bromo, a nitro, a cyano, an acetamido, a carbamoyl, an ureido, an unsubstituted amino, and an amino substituted with one or two alkyls being the same or different and each having 1 to 3 carbon atoms. In a more preferred embodiment, Y¹ and Y² are each Na⁺ or K⁺ and T¹ and T² are each a tolyl group. Most preferred are the Na⁺ or K⁺ salts of p-toluene thiosulfonate and p-toluene sulfinate.

As mentioned above, the emulsion comprises a dye of Class A of structural formula (I) or a dye of Class B of structural formula (II). In these formulae, W₁-W₈ each independently represent an alkyl, acyl, acyloxy, alkoxycarbonyl, carbonyl, carbamoyl, sulfamoyl, carboxyl, cyano, hydroxy, amino, acylamino, alkoxy, alkylthio, alkylsulfonyl, sulfonic acid, aryl, or aryloxy group, any of which may be substituted or unsubstituted, or a hydrogen or halogen atom, and provided further that adjacent ones of W₁-W₈ can bonded to each other via their carbon atoms to form a condensed ring. Class A dyes have structure I and substituents W₁-W₈ are chosen such that J is ≥ 0.0, or, alternatively, Class A dyes can also have the structure II provided substituents W₁-W₈ are chosen such that J is ≥ 0.24 and Class B dyes have structure II and substituents W₁-W₈ are chosen such that J is ≤ 0.10, or, alternatively, Class B dyes can also have structure I provided substituents W₁-W₈ are chosen such that J is ≤ -0.14. Hammett σₚ values are discussed in Advanced Organic Chemistry 3rd Ed., J. March, (John Wiley Sons, NY; 1985). Note that the "ₚ" subscript refers to the fact that the σ values are measured with the substituents in the para position.

Z is a hydrogen or halogen atom or an alkyl group or substituted alkyl group, for example a 1 to 8 carbon atom alkyl group or substituted alkyl group. Preferably Z is a relatively "flat" substituent, such as a hydrogen, halogen or a methyl (substituted or unsubstituted). More particularly Z may be a substituted or unsubstituted methyl or a hydrogen.

Z₁ and Z₂ are independently a 1 to 8 carbon alkyl group (for example, methyl, ethyl, propyl or butyl).

Thus the dye (I) may have the formula (Ia) and the dye of formula (II) may have the formula (IIa) in which:
R₁ and R₂ each independently represent an alkyl group or a substituted alkyl group;
V₂-V₇ are independently H or a 1 to 8 carbon alkyl;
Z is a hydrogen or methyl;
A is a counterion if needed to balance the charge.

Preferably at least one of R₁ or R₂, or both, are alkyl of 1-8 carbon atoms, either of which alkyl may be substituted or unsubstituted. Examples of preferred substituents include acid or acid salt groups (for example, sulfo or carboxy groups). Thus, either or both R₁ or R₂ could be, for example, 2-sulfobutyl, 3-sulfopropyl, sulfoethyl or hydroxyethyl.

In preferred embodiments of the invention, the emulsion contains a dye of Class A and a dye of Class B.

Examples of Class A and B dyes used in photographic elements of the present invention are listed below in Table II but the present invention is not limited to the use of these dyes.

The emulsion preferably also contains an anti-aggregating agent. Preferably the anti-aggregating agent is compound III which has the structure: wherein:
D is a divalent aromatic ring-containing moiety; W₉-W₁₂ each independently represents a hydroxy, a halogen atom, an amino, alkylamino, arylamino, cycloalkylamino, a heterocyclic, heterocyclicamino, arylalkylamino, alkoxy, aryloxy, alkylthio, heterocyclicthio, mercapto, alkylthio, arylthio or aryl group, any of which may be substituted or unsubstituted, or a hydrogen or halogen atom;
G₁ and G₂ each represents N or CH;
Y₁ and Y₂ each represents N or CH provided at least one of G₁ and Y₁ is N and at least one of G₂ and Y₂ is N.

In compound III, D is a divalent aromatic ring-containing moiety, preferably selected from the group consisting of:

In the above, M is a hydrogen atom or a cation so as to increase water solubility, such as an alkali metal ion (Na or K) or an ammonium ion.

Some particular examples of compounds of Formula III above are listed below. Again, the invention is not limited to the use of those specific compounds:

Dyes of Class A and B and compounds of formula III can be prepared according to techniques that are well-known in the art, such as described in Hamer, Cyanine Dyes and Related Compounds, 1964 (publisher John Wiley & Sons, New York, NY) and James, The Theory of the Photographic Process 4th edition, 1977 (Eastman Kodak Company, Rochester, NY). The amount of sensitizing dye that is useful in the invention may be from 0.001 to 4.0 millimoles, but is preferably in the range of 0.01 to 4.0 millimoles per mole of silver halide and more preferably from 0.02 to 0.25 millimoles per mole of silver halide. Optimum dye concentrations can be determined by methods known in the art. Formula III compounds can be typically coated at 1/50 to 50 times the dye concentration, or more preferably 1 to 10 times.

The photographic materials of the present invention can contain tabular grain emulsions such as disclosed by Wey US 4,399,215; Kofron US 4,434,226; Maskasky US 4,400,463; and Maskasky US 4,713,323; as well as US 5,185,239; 5,183,732; 5,178,997; 5,178,998 and 5,217,858. The grain size of the silver halide may have any distribution known to be useful in photographic compositions, and may be either polydipersed or monodispersed.

The silver halide grains to be used in the invention may be prepared according to methods known in the art, such as those described in Research Disclosure, (Kenneth Mason Publications Ltd, Emsworth, England), September, 1994, Number 365, Item 36544 (hereinafter referred to as Research Disclosure I) and James, The Theory of the Photographic Process. These include methods such as ammoniacal emulsion making, neutral or acid emulsion making, and others known in the art. These methods generally involve mixing a water soluble silver salt with a water soluble halide salt in the presence of a protective colloid, and controlling the temperature, pAg, pH values, etc, at suitable values during formation of the silver halide by precipitation. High chloride [1 0 0] tabular emulsions such as described in EP 534,395 can also be used.

The silver halide to be used in the invention may be advantageously subjected to chemical sensitization with compounds such as gold sensitizers (e.g., gold and sulfur) and others known in the art. Compounds and techniques useful for chemical sensitization of silver halide are known in the art and described in Research Disclosure I and the references cited therein.

The photographic materials of the present invention, as is typical, provide the silver halide in the form of an emulsion. Photographic emulsions generally include a vehicle for coating the emulsion as a layer of a photographic element. Useful vehicles include both naturally occurring substances such as proteins, protein derivatives, cellulose derivatives (e.g., cellulose esters), gelatin (e.g., alkali-treated gelatin such as cattle bone or hide gelatin, or acid treated gelatin such as pigskin gelatin), gelatin derivatives (e.g., acetylated gelatin or phthalated gelatin), and others as described in Research Disclosure I. Also useful as vehicles or vehicle extenders are hydrophilic water-permeable colloids. These include synthetic polymeric peptizers, carriers, and/or binders such as poly(vinyl alcohol), poly(vinyl lactams), acrylamide polymers, polyvinyl acetals, polymers of alkyl and sulfoalkyl acrylates and methacrylates, hydrolyzed polyvinyl acetates, polyamides, polyvinyl pyridine, methacrylamide copolymers, as described in Research Disclosure I. The vehicle can be present in the emulsion in any amount useful in photographic emulsions. The emulsion can also include any of the addenda known to be useful in photographic emulsions. These include chemical sensitizers, such as active gelatin, sulfur, selenium, tellurium, gold, platinum, palladium, iridium, osmium, rhenium, phosphorous, or combinations thereof. Chemical sensitization is generally carried out at pAg levels of from 5 to 10, pH levels of from 4 to 8, and temperatures of from 30 to 80°C, as illustrated in Research Disclosure, June 1975, item 13452 and U.S. Patent No. 3,772,031.

The silver halide is sensitized by a dye of Class A and/or a dye of Class B and, optionally, a compound of Formula III by methods known in the art, such as described in Research Disclosure I. The compounds may be added to an emulsion of the silver halide grains and a hydrophilic colloid at any time prior to (e.g., during or after chemical sensitization) or simultaneous with the coating of the emulsion on a photographic element. The resulting sensitized silver halide emulsion may be mixed with a dispersion of color image-forming coupler immediately before coating or in advance of coating (for example, 2 hours). Essentially any type of emulsion (e.g., negative-working emulsions such as surface-sensitive emulsions of unfogged internal latent image-forming emulsions, direct-positive emulsions such as surface fogged emulsions, or others described in, for example, Research Disclosure I) may be used. The above-described sensitizing dyes of Class A and Class B can be used alone, or may be used in combination with other sensitizing dyes, e.g. to also provide the silver halide with sensitivity to wavelengths of light outside the red region or to supersensitize the silver halide.

Other addenda in the emulsion may include antifoggants, especially a heterocyclic mercapto anti-foggant, stabilizers, filter dyes, light absorbing or reflecting pigments, vehicle hardeners such as gelatin hardeners, coating aids, dye-forming couplers, and development modifiers such as development inhibitor releasing couplers, timed development inhibitor releasing couplers, and bleach accelerators. These addenda and methods of their inclusion in emulsion and other photographic layers are well-known in the art and are disclosed in Research Disclosure I and the references cited therein. The emulsion may also include brighteners, such as stilbene brighteners.

The emulsion layer containing silver halide sensitized as described above, can be coated simultaneously or sequentially with other emulsion layers, subbing layers, filter dye layers, interlayers, or overcoat layers, all of which may contain various addenda known to be included in photographic elements. These include antifoggants, oxidized developer scavengers, DIR couplers, antistatic agents, optical brighteners, light-absorbing or light-scattering pigments. The layers of the photographic element can be coated onto a support using techniques well-known in the art. These techniques include immersion or dip coating, roller coating, reverse roll coating, air knife coating, doctor blade coating, stretch-flow coating, and curtain coating, to name a few. The coated layers of the element may be chill-set or dried, or both. Drying may be accelerated by known techniques such as conduction, convection, radiation heating, or a combination thereof.

Photographic materials of the present invention can be black and white photographic elements but are preferably color photographic elements. A color photographic element generally contains three silver emulsion layers or sets of layers (each set of layers often consisting of emulsions of the same spectral sensitivity but different speed): a blue-sensitive layer having a yellow dye-forming color coupler associated therewith; a green-sensitive layer having a magenta dye-forming color coupler associated therewith; and a red-sensitive layer having a cyan dye-forming color coupler associated therewith. Those dye forming couplers are provided in the emulsion typically by first dissolving or dispersing them in a water immiscible, high boiling point organic solvent, the resulting mixture then being dispersed in the emulsion. Suitable solvents include those in European Patent Publication EP-A-O 273,430. Dye-forming couplers are well-known in the art and are disclosed, for example, in Research Disclosure I.

Photographic elements of the present invention may also usefully include a magnetic recording layer as described in Research Disclosure, Item 34390, November 1992.

Photographic elements of the invention can be processed in any of a number of well-known photographic processes utilizing any of a number of well-known processing compositions, described, for example, in Research Disclosure I, or in James, The Theory of the Photographic Process 4th, 1977.

### Photographic Evaluation Example:

A high chloride halide emulsion was precipitated by equimolar addition of silver nitrate and sodium chloride solutions into a well-stirred reactor containing gelatin peptizer and thioether ripener. The resultant emulsion contains cubic shaped grains of 0.38 µm in edgelength size. Emulsions are compared in the presence and absence of ruthenium hexacyanide complex (K₄Ru(CN)₆) as dopant at a level of 75 mppm. Portions of this emulsion were sensitized in the following manner. The emulsion at 40°C was adjusted to a pH of 4.3 with nitric acid and a vAg of 129 with KCl followed by gold and sulfur sensitization. The temperature was increased to 65°C and an antifoggant was added (1-(3-acetamidophenyl)-5-mercaptotetrazole, 0.95 x 10⁻³ mol/molAg) and then combined with compound III-2 (22.3x 10⁻⁵ mol/molAg) and then a soluble bromide was added at 1.1 mole%, the temperature was then decreased to 40°C and the pH of the emulsion was adjusted to 5.6 using NaOH solution. The dyes in Table III were added at 3.64 x 10⁻⁵ mole/silver mole, various levels being used. In Table IV, the dyes were combined in various ratios to yield a total dye coverage of 3.64 x 10⁻⁵ mole/silver mole.

The cyan coupler dispersion contained a cyan image forming coupler ((2-(alpha-(2,4-di-tert-amylphoxy)-butyramido-4,6-dichloro-5-ethyl phenyl)) (0.43g/m², 39.3 mg/ft²) and gelatin (0.85 g/m², 77.0 g/ft²). The coupler dispersion was added to the dye/silver chloride emulsion immediately before coating. The elements also included a gelatin overcoat (1.08 g/m²) and a gelatin undercoat layer (3.23 g/m²). The layers were hardened with bis(vinylsulfonyl)methyl ether at 1.7% of the total gelatin weight. Materials were coated on a resin coated paper support.

To the cyan dispersion was added 1500 mg/m of p-toluene thiosulfonate (TSS) and 150mg/m of p-toluene sulfinate (TS).

To evaluate photographic sensitivity, the elements were exposed to a light source designed to simulate a color negative print exposure. The elements were then processed with RA-4 chemistry through a Colenta processor. This consists of color development (45 sec, 35°C), bleach-fix (45 sec, 35°C), and stabilization or water wash (90 sec, 35°C) followed by drying 60 sec, 60°C).

| **Color Developer** | |
|---|---|
| Lithium salt of sulfonated polystyrene | 0.25 ml |
| Triethanolamine | 11.0 ml |
| N,N-diethylhydroxylamine (85% by wt.) | 6.0 ml |
| Potassium sulfite (45% by wt.) | 0.5 ml |
| Color developing agent (4-(N-ethyl-N-2-methanesulfonylaminoethyl)-2-methylphenylenediaminesesquisulfatemonohydrate | 5.0 g |
| Stilbene compound stain reducing agent | 2.3 g |
| Lithium sulfate | 2.7 g |
| Potassium chloride | 2.3 g |
| Potassium bromide | 0.025 g |
| Sequestering agent | 0.8 ml |
| Potassium carbonate | 25.0 g |
| Water to total of 1 liter, pH adjusted to 10.12 | |

| **Bleach-fix** | |
|---|---|
| Ammonium sulfite | 58 g |
| Sodium thiosulfate | 8.7 g |
| Ethylenediaminetetracetic acid ferric ammonium salt | 40 g |
| Acetic acid | 9.0 ml |
| Water to total 1 liter, pH adjusted to 6.2 | |

| **Stabilizer** | |
|---|---|
| Sodium citrate | 1 g |
| Water to total 1 liter, pH adjusted to 7.2 | |

LIRF is defined as low intensity reciprocity failure measured by calculating the difference between 0.2 sec and 100 sec exposure. A CR unit is defined as 0. 01 logE.

Heat sensitivity was measured by comparing coatings exposed at room temperature (22°C) with coatings exposed on a platen that was heated to 40°C (coatings are equilibrated on the platen for 1.5' before exposing). The difference in speed is taken as a measurement of heat sensitivity. (The magnitude of the heat sensitivity also has an exposure time dependence. Measurements reported here were an 1/10" exposure at 1.0 density point of the D log E curve.)

Emulsions are compared in the presence and absence of ruthenium hexacyanide complex (K₄Ru(CN)₆) dopant at various levels including 50, 60, 75 mppm at various locations within the grain including bands of 75/80%, 75/90%, 80/92%. Both single dyes (Table III) and dye combinations (Table IV) would be preferably used with a tiazinylstilbene compound such as Compound III-2.

**TABLE III**

| Ru Complex | Compound III-2 | Dye | Heat Sensitivity | Heat Sensitivity TSS/TS |
|---|---|---|---|---|
| No | Yes | A-1 | 6.7 | -1.5 |
| No | No | A-1 | 10.6 | 1.3 |
| Yes | Yes | A-1 | 1.8 | -2.8 |
| Yes | No | A-1 | 1.7 | -4.3 |
| No | Yes | B-7 | 4.2 | -2.1 |
| No | No | B-7 | 5.5 | -2.3 |
| Yes | Yes | B-7 | -1.9 | -5.4 |
| Yes | No | B-7 | 1.1 | -6.2 |
| No | Yes | B-1 | 0.5 | -6.3 |
| No | No | B-1 | 3.9 | -3.7 |
| Yes | Yes | B-1 | -2.5 | -7.3 |
| Yes | No | B-1 | -2.7 | -7 |
| No | Yes | B-5 | -0.6 | -7.3 |
| No | No | B-5 | 2.5 | -0.9 |
| Yes | Yes | B-5 | -5.6 | -9.9 |
| Yes | No | B-5 | -2.2 | -5.9 |
| No | Yes | B-4 | 1.7 | -6 |
| No | No | B-4 | 5.6 | -0.5 |
| Yes | Yes | B-4 | -2.5 | -6.1 |
| Yes | No | B-4 | -0.1 | -4.5 |
| No | Yes | B-2 | 3.5 | -2.8 |
| No | No | B-2 | 6.7 | 2.9 |
| Yes | Yes | B-2 | -1 | -3.9 |
| Yes | No | B-2 | 2.3 | -2.3 |
| No | Yes | B-6 | 5.2 | -2.6 |
| No | No | B-6 | 11.3 | 3.9 |
| Yes | Yes | B-6 | -0.5 | -3.9 |
| Yes | No | B-6 | 5.3 | 0 |

The results in Table III show that the heat sensitivity of the red sensitive layer can be modified by the presence of a hexacoordination complex and TSS/TS.

The results in Table IV show that the heat sensitivity of the red sensitive layer can be varied by the presence of differing amounts of a hexacoordination complex and TSS/TS. By modifying the heat sensitivity in this manner, the heat sensitivity of a red sensitive layer can be adjusted to match the heat sensitivity of other layers of a photographic element.

## Claims

1. A silver halide photographic material comprising a red sensitive silver halide emulsion layer, the silver halide of which comprises silver halide grains prepared in the presence of a hexacoordination complex of rhenium, ruthenium or osmium with at least four cyanide ligands and comprising at least 90 mole percent silver chloride, wherein the emulsion contains a thiosulfonate and a sulfinate or seleninate and a dye of Class A and/or Class B:
where,
dye classes A and B have structures I and II. where,
R₁ and R₂ each independently represent an alkyl group or a substituted alkyl group;
X is a counterion, if needed, to balance the charge of the dye;
Z is a hydrogen or halogen atom or an alkyl group or a substituted alkyl group;
Z₁ and Z₂ are each independently a 1-8 carbon alkyl group;
W₁-W₈ each independently represent, an alkyl group, an acyl group, an acyloxy group, an alkoxycarbonyl group, a carbonyl group, a carbamoyl group, a sulfamoyl group, carboxyl group, cyano group, hydroxy group, an amino group, an acylamino group, an alkoxy group, an alkylthio group, an alkylsulfonyl group, sulfonic acid group, aryl group, or aryloxy group, any of which may be substituted or unsubstituted, or a hydrogen or halogen atom, and provided further that adjacent groups can bond to each other via their carbon atoms to form a condensed ring;
and wherein:
Class A dyes have structure I and substituents W₁-W₈ are chosen such that J is ≥ 0.0, where J is defined as the sum of the Hammett σₚ values of W₁-W₈, or, alternatively, Class A dyes can also have the structure II provided substituents W1-W8 are chosen such that J is ≥ 0.24; and
Class B dyes have structure II and substituents W₁-W₈ are chosen independently such that J is ≤ 0.10, or, alternatively, Class B dyes can have structure I provided substituents W₁-W₈ are chosen such that J is ≤ -0.14.

2. A photographic material according to claim 1, wherein the hexacoordination complex is of the formula:
[Q(CN)_{6-y}L_{y}]⁻ⁿ
where:
Q is rhenium, ruthenium, or osmium,
L is a bridging ligand,
y is 0, 1, or 2,
and
-n is -2, -3, or -4.

3. A photographic material according to either of claims 1 and 2, wherein the emulsion contains a thiosulfonate of formula (IV)
T¹―SO₂S―Y¹ (IV)
and a sulfinate compound of formula (Va):
T²―SO₂―Y² (Va)
or a seleninate compound of formula (Vb)
T²―SeO₂―Y² (Vb)
wherein:
Y¹ and Y² are independently selected from the group consisting of a metal ion and wherein D₁, D₂, D₃, and D₄ are independently selected from the group consisting of hydrogen and an alkyl of 1-3 carbon atoms, and T¹ and T² are independently selected from the group consisting of an unsubstituted or substituted alkyl of 1 to 22 carbon atoms, an alkenyl of 2 to 22 carbon atoms, an alkynyl of 2 to 22 carbon atoms, an unsubstituted or substituted aryl group having 6 to 20 carbon atoms, an unsubstituted or substituted 5 to 15-membered heterocyclic group having one or two heteroatoms and a divalent linking group.

4. A silver halide photographic according to any one of the preceding claims, wherein the emulsion contains a thiosulfonate of formula (IV) and a sulfinate of formula (Va).

5. A photographic material according to any one of the preceding claims, wherein the silver halide emulsion further comprises a compound of formula (III): wherein:
D is a divalent aromatic ring-containing moiety;
W₉-W₁₂ each independently represents a hydroxy, a halogen atom, an amino, alkylamino, arylamino, cycloalkylamino, a heterocyclic, heterocyclicamino, arylalkylamino, alkoxy, aryloxy, alkylthio, heterocyclicthio, mercapto, alkylthio, arylthio or aryl group, any of which may be substituted or unsubstituted, or a hydrogen or halogen atom;
G₁ and G₂ each represents N or CH;
Y₁ and Y₂ each represents N or CH provided at least one of G₁ and Y₁ is N and at least one of G₂ and Y₂ is N.

6. A silver halide photographic material according to any one of the preceding claims, wherein the emulsion contains a dye of Class A and a dye of Class B.

7. A silver halide photographic material according to claim 6, wherein the dye of formula (I) is of formula (Ia) and the dye of formula (II) is of formula (IIa): in which:
R₁ and R₂ each independently represent an alkyl group or a substituted alkyl group;
V₂-V₇ are independently H or a 1 to 8 carbon alkyl;
Z is a hydrogen or methyl;
A is a counterion if needed to balance the charge.

8. A silver halide photographic material according to any one of the preceding claims, wherein the silver halide of the emulsion is at least 95 percent silver chloride.

9. A silver halide photographic material according to any one of the preceding claims, wherein the emulsion further comprises a heterocyclic mercapto anti-foggant compound.

## Patentansprüche

1. Photographisches Silberhalogenidmaterial, umfassend eine rotempfindliche Silberhalogenid-Emulsionsschicht, wobei ihr Silberhalogenid Silberhalogenidkörnchen umfaßt, hergestellt in Gegenwart eines Hexakoordinationskomplexes von Rhenium, Ruthenium oder Osmium mit mindestens vier Cyanid-Liganden, und umfassend mindestens 90 Mol-% Silberchlorid, wobei die Emulsion ein Thiosulfonat und ein Sulfinat oder Seleninat und einen Farbstoff der Klasse A und/oder einen Farbstoff der Klasse B enthält:
worin
der Farbstoff der Klasse A und B die Strukturen I und II aufweist: worin
R₁ und R₂ jeweils unabhängig für eine Alkylgruppe oder eine substituierte Alkylgruppe stehen;
X ein Gegenion ist, um, sofern erforderlich, die Ladung des Farbstoffes auszugleichen;
Z ein Wasserstoff- oder Halogenatom oder eine Alkylgruppe oder eine substituierte Alkylgruppe ist;
Z₁ und Z₂ jeweils unabhängig für eine Alkylgruppe mit 1 bis 8 Kohlenstoffatomen stehen;
W₁ bis W₈ jeweils unabhängig für eine Alkylgruppe, eine Acylgruppe, eine Acyloxygruppe, eine Alkoxycarbonylgruppe, eine Carbonylgruppe, eine Carbamoylgruppe, eine Sulfamoylgruppe, eine Carboxylgruppe, eine Cyanogruppe, eine Hydroxygruppe, eine Aminogruppe, eine Acylaminogruppe, eine Alkoxygruppe, eine Alkylthiogruppe, eine Alkylsulfonylgruppe, eine Sulfonsäuregruppe, eine Arylgruppe oder eine Aryloxygruppe, wobei jedwede substituiert oder unsubstituiert sein kann, oder für ein Wasserstoff- oder Halogenatom stehen, und weiterhin mit der Maßgabe, daß benachbarte Gruppen miteinander über ihre Kohlenstoffatome unter Bildung eines kondensierten Ringes verbunden sein können;
und worin
die Farbstoffe der Klasse A die Struktur I aufweisen und die Substituenten W₁ bis W₈ so gewählt sind, daß J ≥ 0,0 ist, wobei J als Summe der Hammett-σₚ-Werte von W₁ bis W₈ definiert ist, oder alternativ die Farbstoffe der Klasse A ebenfalls die Struktur II aufweisen können, mit der Maßgabe, daß die Substituenten W₁ bis W₈ so gewählt sind, daß J ≥ 0,24 ist; und
die Farbstoffe der Klasse B die Struktur II aufweisen und die Substituenten W₁ bis W₈ unabhängig gewählt sind, so daß J ≤ 0,10 ist, oder alternativ die Farbstoffe der Klasse B die Struktur I aufweisen können, mit der Maßgabe, daß die Substituenten W₁ bis W₈ so gewählt sind, daß J ≤ -0,14 ist.

2. Photographisches Material gemäß Anspruch 1, wobei der Hexakoordinationskomplex folgende Formel besitzt:
[Q(CN)_{6-y}L_{y}]⁻ⁿ
worin
Q Rhenium, Ruthenium oder Osmium ist,
L ein Überbrückungsligand ist,
y 0, 1 oder 2 ist, und
-n -2, -3 oder -4 ist.

3. Photographisches Material gemäß einem der Ansprüche 1 und 2, wobei die Emulsion ein Thiosulfonat der Formel (IV)
T¹ - SO₂S - Y¹ (IV)
und eine Sulfinatverbindung der Formel (Va):
T² - SO₂ - Y² (Va)
oder eine Seleninatverbindung der Formel (Vb)
T² - SeO₂ - Y² (Vb)
enthält, worin
Y¹ und Y² unabhängig gewählt sind aus der Gruppe, bestehend aus einem Metallion und worin D₁, D₂, D₃ und D₄ unabhängig gewählt werden aus der Gruppe, bestehend aus Wasserstoff und einem Alkyl mit 1 - 3 Kohlenstoffatomen, und T¹ und T² unabhängig gewählt werden aus der Guppe, bestehend aus unsubstituiertem oder substituiertem Alkyl mit 1 bis 22 Kohlenstoffatomen, einem Alkenyl mit 2 bis 22 Kohlenstoffatomen, einem Alkinyl mit 2 bis 22 Kohlenstoffatomen, einer unsubstituierten oder substituierten Arylgruppe mit 6 bis 20 Kohlenstoffatomen, einer unsubstituierten oder substituierten 5-bis 15-gliedrigen heterocyclischen Gruppe mit einem oder zwei Heteroatomen und einer zweiwertigen Verknüpfungsgruppe.

4. Photographisches Silberhalogenidmaterial gemäß mindestens einem der vorstehenden Ansprüche, wobei die Emulsion ein Thiosulfonat der Formel (IV) und ein Sulfinat der Formel (Va) enthält.

5. Photographisches Material gemäß mindestens einem der vorstehenden Ansprüche, wobei die Silberhalogenidemulsion ferner eine Verbindung der Formel (III) umfaßt: worin
D ein zweiwertiger, einen aromatischen Ring enthaltender Rest ist;
W₉ - W₁₂ jeweils unabhängig für eine Hydroxygruppe, ein Halogenatom, eine Amino-, Alkylamino-, Arylamino-, Cycloalkylamino-, eine heterocyclische, Heterocycloamino-, Arylalkylamino-, Alkoxy-, Aryloxy-, Alkylthio-, Heterocyclothio-, Mercapto-, Alkylthio-, Arylthio- oder Arylgruppe, wobei jedes davon substituiert oder unsubstituiert sein kann, oder für ein Wasserstoff- oder Halogenatom stehen;
G₁ und G₂ jeweils für N oder CH stehen;
Y₁ und Y₂ jeweils für N oder CH stehen, mit der Maßgabe, daß mindestens eines von G₁ und Y₁ N ist und mindestens eines von G₂ und Y₂ N ist.

6. Photographisches Silberhalogenidmaterial gemäß mindestens einem der vorstehenden Ansprüche, wobei die Emulsion einen Farbstoff der Klasse A und einen Farbstoff der Klasse B enthält.

7. Photographisches Silberhalogenidmaterial gemäß Anspruch 6, wobei der Farbstoff von Formel (I) die Formel (Ia) aufweist und der Farbstoff der Formel (II) die Formel (IIa) aufweist: worin
R₁ und R₂ jeweils unabhängig für eine Alkylgruppe oder eine substituierte Alkylgruppe stehen;
V₂ - V₇ unabhängig für H oder ein Alkyl mit 1 bis 8 Kohlenstoffatomen stehen;
Z Wasserstoff oder Methyl ist;
A ein Gegenion ist, um, sofern erforderlich, die Ladung auszugleichen.

8. Photographisches Silberhalogenidmaterial gemäß mindestens einem der vorstehenden Ansprüche, wobei das Silberhalogenid der Emulsion zu mindestens 95% Silberchlorid ist.

9. Photographisches Silberhalogenidmaterial gemäß mindestens einem der vorstehenden Ansprüche, wobei die Emulsion zusätzlich eine heterocyclische Mercaptoverbindung gegen Schleierbildung umfaßt.

## Revendications

1. Produit photographique aux halogénures d'argent comprenant une couche d'émulsion aux halogénures d'argent sensible au rouge dont l'halogénure d'argent comprend des grains d'halogénures d'argent préparés en présence d'un complexe hexacoordiné de rhénium, de ruthénium ou d'osmium avec au moins quatre ligands cyanure et constitué d'au moins 90% en moles de chlorure d'argent, où l'émulsion contient un composé thiosulfonate et un composé sulfinate ou séléninate et un colorant de classe A et/ou de classe B, où :
les colorants de classe A et B sont représentés par les structure I et II. où :
R₁ et R₂ représentent chacun indépendamment un groupe alkyle ou alkyle substitué ;
X est un contre-ion permettant d'équilibrer la charge du colorant, si nécessaire ;
Z est un atome d'hydrogène ou d'halogène ou un groupe alkyle ou alkyle substitué ;
Z₁ et Z₂ représentent chacun indépendamment un groupe alkyle de 1 à 8 atomes de carbone ;
W₁-W₈ représentent chacun indépendamment un groupe alkyle, acyle, acyloxy, alcoxycarbonyle, carbonyle, carbamoyle, sulfamoyle, carboxyle, cyano, hydroxy, amino, acylamino, alcoxy, alkylthio, alkylsulfonyle, acide sulfonique, aryle ou aryloxy, l'un quelconque de ces groupes pouvant être substitué ou non, ou un atome d'hydrogène ou d'halogène, et à la condition supplémentaire que les groupes adjacents puissent être reliés l'un à l'autre par l'intermédiaire de leurs atomes de carbone pour former un cycle condensé ; et où les colorants de classe A sont représentés par la structure I et les substituants W₁-W₈ sont choisis de manière que J soit ≥ 0,0, où J est défini comme étant la somme des valeurs σp de Hammett de W₁-W₈, ou bien, les colorants de classe A sont également représentés par la structure II, à la condition que les substituants W₁-W₈ soient choisis de manière que J soit ≥ 0,24 ; et
les colorants de classe B sont représentés par la structure II et les substituants W₁-W₈ sont indépendamment choisis de manière que J soit ≤ 0,10 ou bien, les colorants de classe B sont représentés par la structure I, à la condition que les substituants W₁-W₈ soient choisis de manière que J soit ≤ -0,14.

2. Produit photographique selon la revendication 1, dans lequel le complexe hexacoordiné est représenté par la formule :
[Q(CN)_{6-y}L_{y}]⁻ⁿ
où :
Q est le rhénium, le ruthénium ou l'osmium,
L est un ligand pontant,
y est 0, 1 ou 2, et
-n est -2, -3 ou -4.

3. Produit photographique selon l'une quelconque des revendications 1 et 2, dans lequel l'émulsion contient un composé thiosulfonate représenté par la formule (IV)
T¹--SO₂S--Y¹ (IV)
et un composé sulfinate représenté par la formule (Va)
T²--SO₂--Y² (Va)
ou un composé séléninate représenté par la formule (Vb)
T²--SeO₂--Y² (Vb)
où :
Y¹ et Y² sont indépendamment choisis parmi le groupe comprenant un ion métallique et où D₁, D₂, D₃ et D₄ sont indépendamment choisis parmi le groupe comprenant l'hydrogène et un groupe alkyle de 1 à 3 atomes de carbone, et T¹ et T² sont indépendamment choisis parmi le groupe comprenant un groupe alkyle substitué ou non de 1 à 22 atomes de carbone, un groupe alcényle de 2 à 22 atomes de carbone, un groupe alkynyle de 2 à 22 atomes de carbone, un groupe aryle substitué ou non de 6 à 20 atomes de carbone, un groupe hétérocyclique substitué ou non de 5 à 15 maillons ayant un ou deux hétéroatomes et un groupe de liaison divalent.

4. Produit photographique aux halogénures d'argent selon l'une quelconque des revendications précédentes, dans lequel l'émulsion contient un composé thiosulfonate représenté par la formule (IV) et un composé sulfinate représenté par la formule (Va).

5. Produit photographique aux halogénures d'argent selon l'une quelconque des revendications précédentes, dans lequel l'émulsion aux halogénures d'argent comprend en outre un composé de formule (III) : où :
D est un radical contenant un cycle aromatique divalent ;
W₉-W₁₂ représentent chacun indépendamment un radical hydroxy, un atome d'halogène, un groupe amino, alkylamino, arylamino, cycloalkylamino, hétérocyclique, hétérocyclique amino, arylalkylamino, alcoxy, aryloxy, alkylthio, hétérocyclique thio, mercapto, alkylthio, arylthio ou aryle, l'un quelconque de ces groupes pouvant être substitué ou non, ou un atome d'halogène ou d'hydrogène ;
G₁ et G₂ représentent chacun N ou CH ;
Y₁ et Y₂ représentent chacun N ou CH, à la condition qu'au moins un des groupes G₁ et Y₁ soit N et qu'au moins un des groupes G₂ et Y₂ soit N.

6. Produit photographique aux halogénures d'argent selon l'une quelconque des revendications précédentes, dans lequel l'émulsion contient un colorant de classe A et un colorant de classe B.

7. Produit photographique aux halogénures d'argent selon la revendication 6, dans lequel le colorant de formule (I) est représenté par la formule (Ia) et le colorant de formule (II) est représenté par la formule (IIa) : où :
R₁ et R₂ représentent chacun indépendamment un groupe alkyle ou alkyle substitué ;
V₂-V₇ sont indépendamment H ou un groupe alkyle de 1 à 8 atomes de carbone ;
Z est l'hydrogène ou un groupe méthyle ;
A est un contre-ion permettant d'équilibrer la charge, si nécessaire.

8. Produit photographique aux halogénures d'argent selon l'une quelconque des revendications précédentes, dans lequel l'halogénure d'argent de l'émulsion est constitué d'au moins 95% de chlorure d'argent.

9. Produit photographique aux halogénures d'argent selon l'une quelconque des revendications précédentes, dans lequel l'émulsion comprend en outre un composé antivoile hétérocyclique de type mercapto.
